

## UNITED STATES PATENT OFFICE.

ROBERT A. HADFIELD, OF SHEFFIELD, ENGLAND.

## MANUFACTURE OF STEEL.

SPECIFICATION forming part of Letters Patent No. 743,715, dated November 10, 1903.

Application filed June 24, 1901. Serial No. 65,801. (No specimens.)

*To all whom it may concern:*

Be it known that I, ROBERT A. HADFIELD, a subject of the King of Great Britain, and a resident of Sheffield, county of York, England, have invented an Improvement in the Manufacture of Steel, of which the following description is a specification.

As a result of the decarbonizing and desilicizing process in the production of steel by various pneumatic methods now commonly practiced the fluid metal becomes permeated with gases, and consequently very unsound, whether owing to the presence of dissolved gases, occluded oxygen, or other cause is not definitely known, and with the object of remedying this condition it is usual to make additions of silicon, aluminium, or other alloys of metals. While such additions are of some service, it is doubtful whether by their use the oxygenated fluid metal is in practice ever restored to its highest value.

My present invention has for its object a novel method of obviating or mitigating the evil hereinbefore referred to, and in accordance therewith I control the oxidation of the molten metal during the process of its conversion into steel by the introduction of manganese to the charge, meaning by the term "conversion process" the process of converting fluid pig-iron and scrap or other mixtures into steel. The introduction or addition of the manganese is made in a practically continuous manner or at short intervals throughout the blow or charge or during the latter portion thereof or it may be added after the disappearance of carbon from the charge, provided the blow is continued after such addition sufficiently to practically complete the oxidation of all the added manganese. By this method of treatment I obtain a decarbonized and desilicized iron exceedingly sound as compared with ordinary samples obtained in the usual manner, and, furthermore, the use of expensive quieting additions, such as aluminium, may be largely or entirely dispensed with and a product obtained resembling the best qualities of crucible steel much more than does the product ordinarily obtained.

To the product obtained in accordance with my invention the usual physics may be added,

if desired, or the usual steel-making additions; but when very soft steel is required such additions may be dispensed with.

In some cases—for example, when treating by pneumatic processes—I add silicon by the introduction of ferrosilicon or other alloy of silicon during the blow, so as to increase the temperature, and, on the other hand, to reduce the temperature I sometimes add white pig-iron or other similar product. Use may be also made of siliconspeigel where a combined silicon and manganese is desired, or a spiegeleisen may be used.

My invention may be practiced in the production of steel in various ways. As one example, assuming that a charge is being treated by any of the pneumatic processes for making steel, if manganese be added thereto by the introduction of ferromanganese containing, say, eighty (80) per cent. of manganese the decarbonized and desilicized iron will, as compared with products obtained in the usual manner, be much freer from the occluded gases, the product being comparatively sound and much less red-short. A charge so prepared, when steel-making additions are being added, will be much sounder than one prepared without the employment of my invention.

One practical mode of carrying out my invention is to add the ferromanganese or other manganese alloy in a practically continuous manner—*i. e.*, at short intervals—throughout the blow or charge, so as to keep the oxidation under control. Thus, for example, in a five-ton heat I may make a total addition of, say, eighty (80) pounds of eighty (80) per cent. ferromanganese, this quantity being added by introducing portions of it at intervals extending over the entire duration of the blow—say every one or two minutes, more or less. Another mode of procedure is to add similar or greater quantities or smaller total quantities of eighty (80) per cent. ferromanganese during only a portion of the blow. Thus, for example, there might be added during the latter part of the blow say forty (40) pounds of ferromanganese, distributed in equal quantities, or approximately so, at intervals of time, in lieu of making any addition of manganese during the first of the blow.

The quantity of manganese added, as also the time or times at which the addition is made, may be varied according to requirement. Thus in some cases the addition might 5 be made as late as during the last quarter only of the entire duration of the blow. Manganese might also, for the purposes of my invention, be added after completion of the ordinary blow—that is, after the disappearance 10 of carbon from the charge—care being taken to continue the blow after addition of the manganese sufficiently to complete or practically complete the oxidation of all the added manganese. Usually, however, it will 15 be found preferable to make the addition of manganese before all the carbon has been oxidized, since the dropping of the carbon flame will then afford a satisfactory indication not only that the carbon has disappeared, 20 but also that the manganese has been oxidized, or nearly so.

The steel obtained can be poured into ingots or castings and treated in the usual manner.

25 It is to be noted that mere presence of manganese in the bath before commencement of the process of conversion into steel will not give the desired result, because the manganese in this case will be oxidized too soon, 30 whereas according to my invention the oxidation can be kept under control during the whole of the blow with minimum expenditure of manganese, besides which the manganese additions tend to reduce the percentage 35 of sulfur present, so that even when

using comparatively cheap stock satisfactory products may be obtained.

Having fully described my invention, what I claim as new, and desire to secure by Letters Patent, is—

1. In the art of steel-making by the pneumatic method, the process of controlling the oxidation of the molten metal during the conversion thereof into steel, which consists in making successive introductions of manganese to the charge subsequent to the commencement and before the completion of the blow.

2. In the art of steel-making by the pneumatic method, the process of controlling the oxidation of the molten metal during the conversion thereof into steel, which consists in making successive additions of manganese, at short intervals, to the charge during the blow.

3. In the process of steel-making by the pneumatic method, adding a temperature-changing agent during the blow to vary the temperature of the charge, and introducing manganese at intervals after the commencement of the blow, and continuing such additions during the blow to control the oxidation of the charge.

In testimony whereof I have signed my name to this specification in the presence of two subscribing witnesses.

ROBERT A. HADFIELD.

Witnesses:

A. C. TEVIS,  
LUTHER J. PARR.